

[72] Inventor **Rolf Mack**  
Binningen Baselland, Switzerland  
[21] Appl. No. **715,517**  
[22] Filed **Mar. 25, 1968**  
[45] Patented **Nov. 2, 1971**  
[73] Assignee **Sandoz Ltd., also known as Sandoz A.G.**  
**Basel, Switzerland**  
[32] Priority **Apr. 7, 1967**  
[33] **Switzerland**  
[31] **4994/67**

[54] **DYEING PROCESS FOR BLENDS OF CELLULOSIC  
AND POLYESTER FIBRES**  
14 Claims, No Drawings  
[52] U.S. Cl. .... **8/21 C,**  
8/14, 8/54.2, 8/179, 8/163

[51] Int. Cl. .... **D06P 3/82**  
[50] Field of Search. .... **8/14, 54.2,**  
**179, 21**  
*Primary Examiner—George F. Lesmes*  
*Assistant Examiner—H. Wolman*  
*Attorney—Irwin Morton Aisenberg*

**ABSTRACT:** A process for dyeing blends of natural or regenerated cellulosic fibers and polyester fibers with reactive and disperse dyes, wherein the cellulosic component of the blend is dyed first with reactive dyes at temperatures in the range of 40° to 100° C. and in the pH range of 8.5 to 13, after which the pH is adjusted to 4-7, the disperse dye added and the polyester component of the blend dyed.

## **DYEING PROCESS FOR BLENDS OF CELLULOSIC AND POLYESTER FIBRES**

The dyeing of blends of cellulosic and polyester fibers with reactive and disperse dyes by a one-bath process is already known (cf. French Pat. No. 1 377 781). This process, in which not more than 5 grams of a basic fixing agent per litre dyeliqour are used, is timesaving compared with a two-bath procedure and consequently the output is greater for a given period of time. However the process requires that the dyes, more particularly the disperse dyes, are stable to alkalis, and it functions satisfactorily only with selected disperse dyes.

It has now been found that this great disadvantage can be overcome by conducting the one-bath process in two stages, the blend being dyed in the first stage with reactive dyes under alkaline conditions and at temperatures up to 100° C. and in the second stage with disperse dyes under weakly acid conditions, either at about 100° C. in the presence of a carrier or above 100° C. under static pressure.

Thus the distinctive feature of this new process for dyeing blends of natural or regenerated cellulosic fibers and polyester fibers with reactive and disperse dyes is that the cellulosic component is dyed initially with reactive dyes in the presence of at least one neutral salt and not more than 20 grams of a basic fixing agent per liter dyeliqour at a temperature in the range of 40° to 100° C. and at a pH of 8.5 to 13 or preferably 10 to 13, following which the pH of the bath is adjusted to 4 to 7 the disperse dye added and the polyester component dyed.

Cotton, linen, hemp, jute and ramie may be mentioned as examples of natural cellulosic fibers which may be present in the blend, while viscose filament and spun rayon and cuprammonium rayon are examples of regenerated cellulosic fibers. These materials can be dyed by the new process, which belongs to the group of exhaustion dyeing processes, in the form of monofilament or multifilament, yarns, sliver, woven fabrics, knitted goods and other textiles. Cellulosic monofilament and multifilament yarns are blended with polyester yarns, generally those spun from the polyesters formed by polycondensation of terephthalic acid and glycols, preferably ethylene glycol or 1,4-bis-(hydroxymethyl)-cyclohexane, and the blend is dyed either in the yarn form or after weaving or knitting in piece form. For one-bath dyeing the dyebath is set with reactive dyes for the natural or regenerated cellulosic fiber and after the dyeing of the cellulosic fiber with disperse dyes for the polyester component of the blend.

The suitable reactive dyes are those bearing a substituent which forms a chemical linkage with the fiber, for example a halogen atom readily cleavable as an anion, preferably a chlorine or bromine atom, or a group cleavable as an anion, e.g.  $-\text{O}-\text{SO}_3\text{H}$ , or a C—C multiple linkage capable of additive reaction. These dyes may belong to the azo, anthraquinone, phthalocyanine or nitro series and may bear any of the following groups or radicals:

- a. at least one dichloro-, trichloro-, dibromo- or tribromo-pyrimidyl, 2,4-dichloro-6-methyl, 2,4-dibromo-6-methyl, 2,4-dichloro- or 2,4-dibromo-phrimidyl-5-methylene group bound through an oxygen or sulfur atom or through an imino group which may itself be substituted;
  - b. a group of the formula



where Hal stands for chlorine or bromine, X for an oxygen or sulfur atom or an imino group which may be substituted and Z for hydrogen or an alkyl, cycloalkyl, aryl or aralkyl radical which may be substituted, said group of formula (I) being bound through an oxygen or sulfur atom or an imino group which may in turn be substituted:

- c. a 4,6-dichloro- or 4,6-dibromo-1,3,5-triazinyl-2-group which is bound through an oxygen or sulfur atom or an imino group which may be substituted;

d. the group  $-\text{SO}_2-\text{CH}_2-\text{CH}_2-\text{O}-\text{SO}_3\text{H}$  or  $-\text{SO}_2-\text{CH}_2-$ ;

e. the group  $-\text{SO}_2-\text{NH}-\text{CH}_2-\text{CH}_2-\text{O}-\text{SO}_3\text{H}$ .

f. a 2,3-dichloroquinoxalyl-6-carbonyl, 4-(4',5'-dichloropyridazon-6'-yl-1')-phenylcarbonyl or  $\beta$ -(4',5'-dichloropyridazon-6'-yl-1')-propionyl group bound through an imino group which may be substituted;

g. a  $\beta$ -chloro-,  $\beta$ -bromo- or  $\beta$ -sulphato-propionyl group or acrylyl group bound through an imino group which may be substituted.

15 Dyes of the aforementioned type are described for example in the following patent specifications:

- a. French Pat. No. 1,221,621 (dichloro- or dibromo-pyrimidylamino radical)
  - Belgian Patent 578,742 and Austrian Patent 214,546 (trichloro- or tribromo-pyrimidylamino radical)
  - Belgian Patent 589,972 (2,4-dichloro- or 2,4-dibromo-6-methylpyrimidyl-5-methylene-amino radical)
  - b) Belgian Patent 559,944; 559,945; 560,734; 563,864; 560,791-795 (4-halogeno-1,3,5-triazinyl-2-radical substituted in the 6-position)
  - c. French Pat. No. 1,180,974 (4,6-dichloro- or 4,6-dibromo-1,3,5-triazinyl-2 radical)
  - d. British Pat. No. 981,195  $\text{--SO}_2\text{--CH}_2\text{--CH}_2\text{O--SO}_3\text{H}$  or  $\text{--SO}_2\text{--CH}_2\text{CH}_2$  radical
  - e. French Pat. No. 1,192,412  $\text{--SO}_2\text{--NH--CH}_2\text{--CH}_2\text{--O--SO}_3\text{H}$  radical
  - f. French Pat. Nos. 1,318,843 1,269,147 2,3-dichloroquin-oxalyl-6-carbonyl radical



or



radical;

- g. Belgian Pat. No. 565,279  $\beta$ -chloropropionyl or acrylyl radical.

The preferred reactive dyes are those which exhaust on cellulosic fibers to an acceptable degree for a bath containing a neutral salt. This practical rule is well known to the textile colorist and its application in the present process can be illustrated by saying that dyes are used which exhaust on the cellulosic fibers in the presence of about 20 grams or more of sodium sulfate or sodium chloride per liter of the dyebath.

Reactive dyes of special interest for the process are those which bear one of the reactive groups defined in (a) or (b) above and which are absorbed by cellulosic fibers in the presence of about 40 to 80 grams of sodium sulfate or sodium chloride per liter of dyebath at pH 10 to 13 to a degree which leaves the bath practically exhausted. The disperse dyes used may belong, for example, to the monoazo, disazo, anthraquinone, nitro, styryl or quinophthalone series. These form stable dispersions in the weakly to very weakly acid dyebaths at the stated dyeing temperatures and have good affinity for polyester fibers and good light fastness. Their melting points are almost invariably higher than 100° C. and in general are superior to 140° C. [see the table in the *Journal of the Society of Dyers and Colorists* 70, pages 69-71 (1954) and the

- 70 Discussion in 74, page 389, (1958)]. The water solubility of these dyes at 80° C. is in general not greater than 100 milligrams per liter, i.e. 1:10,000 [Journal of the Society of Dyers and Colorists 70, 69-71 (1954)] and is preferably between about 0.2 and 50 milligrams per liter. The dyes contain no ionizing groups, such as  $-\text{COOH}$  and  $-\text{SO}_3\text{H}$ , and no groups

which are readily converted into  $-\text{COOH}$  or  $-\text{SO}_3\text{H}$  groups under the dying conditions.

Examples of disperse dyes of the aforescribed nature are described in the following journals and books:

Journal of the Society of Dyers & Colourists 70, 68-75, 5  
1954; 75, 141-147, 1959;  
Canadian Textile Journal, May 1, 1959, 49-59;  
American Dyestuff Reporter 48, 14,35-47 (1959); 49,  
15,600-605 (1960);  
Ullmann, Enzyklopädie der technischen Chemie, Vol. 10  
3 726-8, 1953, (anthraquinone dyes); Vol. 4 128-9,  
1953 (azo dyes);  
French Patents 1 167 704; 1,177,837; 1,207,000;  
1,220,194; 1,222,237; 1,226,501; 1,237,149; 1,264,972;  
1,280,998; 1,281,023; 1,291,988; 1,261,580;  
French Additional Patents 75,125; 76,452; 78,167; (Azo 15  
dyes);  
French Patents 1,163,682; 1,218,936; 1,225,449 (anthra-  
quinone dyes);  
French Patent 1,129,460; British Patent 1,040,607  
(nitro dyes);  
German Patent 677,641; British Patent 843,644 (styryl  
dyes).

Fixing agents are used which have a pH value of at least 8.5 in aqueous solution at 20° C., for example sodium hydroxide, potassium hydroxide, lithium hydroxide, sodium carbonate, potassium carbonate, sodium or potassium bicarbonate, trisodium phosphate, or a sodium or potassium silicate with a molecular ratio of  $\text{SiO}_2:\text{Na}_2\text{O}$  or  $\text{SiO}_2:\text{K}_2\text{O}$  of 1:1 to 3.5:1, e.g. a sodium or potassium metasilicate or sodium water-glass.

Suitable neutral salts include sodium chloride or sulfate and potassium chloride or sulfate.

The cellulosic component of the blend is dyed at 40° to 100° C. or, preferably, at 80°-95° C. at a goods to liquor ratio of about 1:4 to 1:30 or, preferably, 1:5 to 1:15. The amount of basic fixing agent used must be so calculated that the entire amount of hydrogen halide liberated in fixation is bound and the pH of the bath does not fall below 10. At short liquor ratios, e.g. 1:4 to about 1:8, and high reactive dye concentrations, e.g. 5-10 percent on the weight of the goods, the amount of basic fixing agent per liter must be greater than the amount used for dyeing at medium or long liquor ratios. Generally, an addition of 2 to 20 grams of potassium or sodium carbonate or trisodium phosphate or 0.2 to 1.2 grams of potassium or sodium hydroxide per liter dyebath suffices. The dyeing time is about 15 minutes at least and generally 30 to 60 minutes; it depends on the reactive dye used, the nature of the cellulosic component of the blend, the dyeing temperature, the alkali concentration and the alkalinity of the dyebath.

For pale dyeings which require less than 1.0 to 1.5 percent (the weight of the goods) of a solid disperse dye preparation consisting of about 30-35 percent dye, about 50 percent dispersing agent and 15-20 percent standardizing material, it is advisable to add about 0.5 to 2.0 grams per liter of a dispersing agent to the dyebath prior to the addition of the dye; this recommendation also applies when disperse dyes in liquid form are used.

After the cellulosic component has been dyed to shade, the pH of the bath is adjusted to 4 to 7 or, preferably, 5-6.5. For this purpose any of the acids commonly used in dyeing can be employed, such as acetic, sulfuric or phosphoric acid, or an acid salt, such as sodium or, potassium hydrogen sulfate, or preferably, a primary phosphate of formula  $\text{MeH}_2\text{PO}_4$ , where Me represents an alkali metal (sodium, potassium), ammonia or a low molecular alkylammonium radical ( $\text{CH}_3-\text{NH}_3^+$ ,  $(\text{CH}_3)_2\text{NHB}_2^+$ , etc.). When the alkali has been neutralized and the pH adjusted to 4 to 7, the disperse dye is added, for example, in aqueous dispersion or in solution in a suitable organic solvent or mixture of such solvents. The polyester component is then dyed in the presence of a carrier, for example a chlorinated benzene, 1-hydroxy-2-phenylbenzene or a mixture of terephthalic acid dimethyl ester, benzoylaminobenzene and sodium sulfate, at 95°-100° C. or at the boil. Alternatively, it can be dyed in the absence of carrier 75

at temperatures about 100° C., e.g. 110°-140° C. or, preferably, 120°-130° C., under static pressure.

The dyed yarn or fabric is rinsed, washed off with soap and sodium carbonate or with an anionic or nonanionic detergent and sodium carbonate as required, then rinsed again and dried. When the carrier used is 1-hydroxy-2-phenylbenzene, it is advisable to expose the dried yarn or fabric to dry heat for a short time, for example for 1 minute at 190°-200° C., in order to eliminate all traces of this compound. The dyeings are of full shade and have good fastness to light, sublimation, dry heat treatments and dry cleaning, together with excellent fastness to water, perspiration, rubbing and washing at temperatures up to 100° C.

In comparison with the process described in French Pat. specification No. 1,377,781 the present process has the advantage that any desired disperse dyes can be used, including those which are not stable to alkaline solutions on heating. For example, the dyes whose formulas are shown below give excellent results when applied by the present process, whereas in the known process the dye marked ④ is entirely decomposed and dye ② builds up only to weak depth on the polyester fiber, probably owing to saponification of the ester group to the  $-\text{COOH}$  group:



British Patent 843,644, Example 1, paragraph 5

and



British Patent 841,927, Example 33

In the examples that follow the parts and percentages are by weight and the temperatures in degrees centigrade.

#### EXAMPLE 1

The bath is set at 60° with 500 parts of water, 1 part of sodium 3-nitrobenzenesulphonate, 20 parts of calcined sodium sulfate, 2.5 parts of calcined sodium carbonate and 1 part of the dye of the formula



100 parts of a blend yarn consisting of 33 parts of regenerated cellulosic fiber and 67 parts of polyester fiber of the polyethylene-terephthalate type are entered into the bath. The bath is circulated for 15 minutes at 60°, its temperature then raised to 85° in 30 minutes and this temperature held a further 30 minutes with constant circulation. At this point 15 parts of primary sodium phosphate ( $\text{NaH}_2\text{PO}_4 \cdot 2\text{H}_2\text{O}$ ) and 2 parts of a dye preparation of 35 percent of the dye 2,6-dichloro-4-nitro-4'-( $N$ -β-cyanethyl-  $N$ -β-acetoxyethylamino)-1,1'-azobenzene ②, 25 percent sodium dinaphthylmethanedisulphonate, 20 percent sodium cetyl sulfate and 20 percent calcined sodium sulfate are added. The bath is raised to 130° over the next 30 minutes or so and dyeing is continued at this temperature for 1 hour. It is then cooled to 60° in 20 minutes and the dyed yarn

is rinsed with hot water, soaped for 20 minutes at the boil, rinsed again in hot and cold water and dried. The resulting yellow-orange dyeing is fast to light and has very good wash fastness.

## EXAMPLE 2

100 parts of a blend yarn consisting of 33 parts of cotton and 67 parts of polyester fiber are entered into a bath at 60° composed of 1500 parts of water, 1.5 parts of sodium 3-nitrobenzenesulphonate, 60 parts of calcined sodium sulfate, 7.5 parts of trisodium phosphate ( $\text{Na}_3\text{PO}_4 \cdot 10\text{H}_2\text{O}$ ) and 0.9 part of the dye of the formula



The circulating liquor is held at 60° for 15 minutes and then raised to 85° in 30 minutes. Dyeing is continued for 30 minutes at this temperature, after which time are added 9.5 parts of primary sodium phosphate and 2 parts of a dye preparation made up of 35 percent of the dye 2-chloro-4-nitro-4'-(N-β-cyanethyl-N-β-acetoxyethylamino)-1,1'-azobenzene ④, 25 percent sodium dinaphthylmethanedisulphonate, 20 percent sodium cetyl sulfate and 20 percent calcined sodium sulfate. The dyeing cycle is brought to a close as described in example 1. The scarlet dyeing obtained has very good light and wash fastness.

## EXAMPLE 3

100 parts of a blend yarn spun with 67 parts of a polyester fiber of the type named in example 1 and 33 parts of regenerated cellulosic fiber are entered into a bath consisting of 3,000 parts of water, 6 parts of sodium 3-nitrobenzenesulphonate, 120 parts of calcined sodium sulfate, 1.2 parts of sodium hydroxide and 0.9 part of the dye of the formula



The dyeliqour is circulated for 15 minutes at 60° and then raised to 85° in 30 minutes. The blend yarn is dyed at this temperature for a further 30 minutes. After this time 10 parts of primary sodium phosphate are added to the circulating liquor, followed by 1.8 parts of a dye preparation consisting of 35 percent brominated 1,5-dihydroxy-4,8-diaminoanthraquinone ⑥, 25 percent sodium dinaphthylmethanedisulphonate, 20 percent sodium cetyl sulfate and 20 percent calcined sodium sulfate. The bath is raised to 130° in 30 minutes and held at this temperature for 45 minutes. Over the next 20 minutes it is cooled to 60° and subsequently the dyed yarn is rinsed with hot water, soaped for 20 minutes at the boil, rinsed again with hot and cold water and dried. A level blue dyeing is obtained which is fast to light and wet treatments.

The brominated 1,5-dihydroxy-4,8-diaminoanthraquinone of the aforestated dye preparation can be replaced by the dye 2-hydroxy- 5-methyl-4'-benzoylamino-1,1'-azobenzene 7 or the dye of the formula



Alternatively, dye 5 can be replaced by dye 1 to give two-color effects on the blend with a green overall appearance.

## EXAMPLE 4

15 A dyebath is set at 60° with 1,500 parts of water, 1.5 parts of sodium 3-nitrobenzenesulphonate, 90 parts of calcined sodium sulfate, 0.9 part of sodium hydroxide and 1.8 parts of the dye of the formula

Trichloropyrimidyl-HN-



35 100 parts of a blend yarn consisting of 33 parts of cotton and 67 parts of a polyester fiber of the type mentioned in example 1 are entered into the bath, which is then circulated for 30 minutes while the temperature is raised to 90°. This temperature is maintained for a further 30 minutes. At this point the bath is set for polyester dyeing with 7 parts of primary sodium phosphate and 3.8 parts of a dye preparation composed of 30 percent 2-bromo-4,6-dinitro-2'-acetylaminio-4'-(N,N-bis (β-acetoxyethyl)-amino) -5'-ethoxy-1,1-azobenzene 10, 30 percent sodium dinaphthylmethanedisulphonate, 20 percent sodium cetyl sulfate and 20 percent calcined sodium sulfate. 40 45 This second stage of dyeing is carried out as detailed in example 1. A level navy dyeing is obtained which is fast to light and wet treatments.

## EXAMPLE 5

100 parts of a blend yarn composed of 33 parts of cotton and 67 parts of a polyester fiber of the type named in example 1 are entered into a bath consisting of 1,500 parts of water at 60°, 1.5 parts of sodium 3nitrobenzenesulphonate, 60 parts of calcined sodium sulfate, 0.75 part of sodium hydroxide and 0.9 part of the dye of the formula



The circulating liquor is held at 60° for 15 minutes, raised to 95° in 30 minutes and held at this temperature for 1 hour for cellulosic fiber dyeing. Subsequently the bath is set with 670 parts of primary sodium phosphate and 1.8 parts of a dye preparation of 35 percent 2-cyano-4-nitro-4'-(N-ethyl-N-β-cyanethylamino)-1,1'-azobenzene 12, 30 percent sodium dinaphthylmethanedisulphonate, 20 percent sodium cetyl sulfate and 15 percent calcined sodium sulfate. Dyeing is finalized as detailed in example 1 and gives a ruby dyeing which is fast to light and wet treatments.

## EXAMPLE 6

A dyebath is prepared at 60° with 2,000 parts of soft water, 4 parts of 3-nitrobenzenesulphonate, 80 parts of calcined sodium sulfate, 10 parts of trisodium phosphate ( $Na_3PO_4 \cdot 10H_2O$ ) and 1 part of the dye of the formula



100 parts of a blend yarn consisting of 33 parts of regenerated cellulose fiber and 67 parts of polyester fiber are entered into the bath, which is circulated for 15 minutes at 60°, after which the temperature is increased to 85° in 30 minutes. Dyeing is continued for 30 minutes at this temperature. At this point further additions are made as follows: 8 parts of 60 percent acetic acid, 2 parts of sodium dinaphthylmethanedisulphonate, 4.5 parts of the sodium salt of 1-hydroxy-2-phenylbenzene in aqueous solution, 0.5 part of a highly sulfonated castor oil and 1.5 parts of a dye preparation composed of 35 percent dye 4 (example 2), 25 percent sodium dinaphthylmethanedisulphonate, 20 percent sodium cetyl sulfate and 20 percent calcined sodium sulfate. The bath is raised to the boil in 30 minutes and dyeing is conducted for 1-2 hours at this temperature. Subsequently the dyed yarn is removed, rinsed with hot water, soaped at the boil for at least 20 minutes in a weakly alkaline bath, rinsed again with hot and cold water and dried. The orange-red dyeing is fast to light and washing.

## EXAMPLE 7

A dyebath is prepared in a high temperature dyeing machine with 1,500 parts of water, 3 parts of sodium 3-nitrobenzenesulphonate, 60 parts of calcined sodium sulfate, 7.5 parts of trisodium phosphate ( $Na_3PO_4 \cdot 10H_2O$ ), 0.8 part of the dye of the formula



and 0.08 part of dye 1 (example 1). At 60° 100 parts of a blend yarn consisting of 67 parts of polyester fiber and 33 parts of regenerated cellulose fiber are introduced into the bath. It is then circulated for 15 minutes at 60° and over the next 30 minutes is raised to 85°, the blend being dyed for a further 30 minutes at this temperature. Circulation is continued while the bath is set with the additions for the second stage of dyeing: 3.8 parts of 60 percent acetic acid, 1.5 parts of sodium dinaphthylmethanedisulphonate and 1 part of a mixture of 25 percent sodium dinaphthylmethanedisulphonate, 20 percent sodium cetyl sulfate, 20 percent anhydrous sodium sulfate, 17 percent dye 4 (example 2) and 18 percent dye of the formula



The bath is raised to 130° in 30-40 minutes and held at this temperature for 45 minutes. It is then cooled to 80° and the dyed blend is removed, rinsed with hot water, soaped for 20 minutes at the boil, rinsed again with hot and cold water and dried. A level scarlet dyeing is obtained which is extremely fast to light and wet treatments.

## EXAMPLE 8

10 A dyebath is prepared with 1,500 parts of water, 3 parts of sodium 3-nitrobenzenesulphonate, 15 parts of trisodium phosphate ( $Na_3PO_4 \cdot 10H_2O$ ), 75 parts of calcined sodium sulfate and 0.8 part of the dye of the formula



15 At 30° 100 parts of a blend yarn consisting of 33 parts of regenerated cellulose fiber and 67 parts of polyester fiber are entered into the bath and turned regularly for 15 minutes at the same temperature, after which the bath is raised to 60° in 30 minutes and the yarn dyed for a further 45 minutes at this temperature. At this point the following additions are made: 7.5 parts of 60 percent acetic acid, 0.75 part of sodium dinaphthylmethanedisulphonate and 2 parts of the dye preparation used in example 3 (dye 6). Over the next 30-40 minutes the bath is raised to 130° under static pressure and the dyeing process is brought to a close in 1 hour at this temperature. The dyed yarn is removed from the bath, rinsed with water, soaped at the boil for 20 minutes in a neutral or weakly alkaline bath, rinsed again with hot and cold water and finally dried. The blue dyeing is fast to light and very fast to washing.

## EXAMPLE 9

20 100 parts of a blend yarn composed of 67 parts of polyester fiber and 33 parts of viscose staple fiber are entered at 40° into a bath of 1,500 parts of water and 2 parts of the dye of the formula



25 50 Over the next 30 minutes 75 parts of calcined sodium sulfate are added and over the subsequent 30 minutes 18 parts of trisodium phosphate ( $Na_3PO_4 \cdot 10H_2O$ ), in both cases in three portions. After the addition of the final portion of trisodium phosphate dyeing is conducted for 90 minutes at 40°. The circulating bath is then set for polyester dyeing with 9 parts of 60 percent acetic acid and 5 parts of a dye preparation formulated with 30 percent 1-amino-2-phenoxy-4-hydroxyanthraquinone 18, 60 percent sodium dinaphthylmethanedisulphonate and 10 percent sodium lignin-sulphonate. The bath temperature is increased to 130° in 30-40 minutes and this temperature is maintained for 60 minutes. Subsequently the bath is cooled to 80°-90° and dropped. After a short rinse with hot water the dyed yarn is soaped at the boil for 15-30 minutes, rinsed again with hot and cold water and dried. It is dyed in a brilliant red which is fast to light and wet treatments.

## EXAMPLE 10

30 75 100 parts of a blend yarn spun with 67 parts of polyester fiber and 33 parts of viscose staple fiber are entered at 50° into

a dyebath set with 1,500 parts of water and 0.7 part of the dye of the formula



After 10 minutes 60 parts of calcined sodium sulfate are added to the circulating bath and after a further 10 minutes 9.75 parts of sodium bicarbonate. Dyeing is continued for 90 minutes at 50°, following which the bath is set with 11.6 parts of 60 percent acetic acid and after brief intermediate circulation with 2 parts of a dye preparation composed of 25 percent 1-amino-4-hydroxy-2-methoxy-ethoxy-ethoxy-xanthraquinone 20, 50 percent sodium dinaphthylmethanedisulphonate and 25 parts sodium ligninsulphonate. Over the next 30-40 minutes the bath temperature is increased to 130° and the dyeing cycle completed in 60 minutes at this temperature. The bath is then cooled and dropped, the dyed material rinsed with hot water, soaped at 100° for 20 minutes, rinsed again with hot and cold water and dried. The resulting red dyeing is fast to light and wet treatments. The following table contains further examples of dyeing in accordance with the present process, for which the procedures and conditions detailed in examples 1 to 10 were employed. In the following the composition of the blend fabric dyed in these examples and the additions to the dyebaths are set forth.

**Blend Fabric:**

33 percent Cotton/67 percent polyethylene terephthalate fiber in examples 17, 26, 28 and 37

33 percent Viscose filament/67 percent polyethylene terephthalate fiber in examples 11 and 29

33 percent Viscose staple fiber/67 percent polyethylene terephthalate fiber in examples 12 to 16, 19, 22, 27, 31, 32, 33 and 36.

50 percent Cotton/50 percent polyethylene terephthalate fiber in examples 18, 25, and 30.

50 percent Viscose staple fiber/50 percent polyethylene terephthalate fiber in examples 20, 21 and 24.

33 percent Cotton/67 percent polyester fiber from terephthalic acid and 1,4-di-(hydroxymethyl)-cyclohexane in examples 23, 34 and 35

### Neutral Salt (termed "salt" in the table)

**NaCl** in examples 13, 25 and 35 to 37  
**KCl** in examples 14, 26, 30 and 34  
**Na<sub>2</sub>SO<sub>4</sub>** in examples 11, 12, 17 to  
**K<sub>2</sub>SO<sub>4</sub>** 24, 27, 28 and 31 to 33  
**CaSO<sub>4</sub>** in examples 15, 16 and 20

### Basic compounds (termed "alkali" in the table)

| Basic compounds (termed "alkali" in the table) |                       |
|------------------------------------------------|-----------------------|
| LiOH                                           | in examples 11        |
| NaOH                                           | in examples 13 and 36 |
| KOH                                            | in examples 34        |
| Na <sub>2</sub> CO <sub>3</sub>                | in examples 25 and 37 |

|                                  |                                                    |
|----------------------------------|----------------------------------------------------|
| $K_2CO_3$                        | in examples 14, 16 and 30                          |
| $Li_2CO_3$                       | in examples 12                                     |
| $NaHCO_3$                        | in examples 18 and 20                              |
| $KHCO_3$                         | in example 19                                      |
| $Na_2SiO_3 \cdot 9H_2O$          | in example 23                                      |
| $K_2SiO_3$                       | in example 26                                      |
| $Na_2B_4O_7 \cdot 10H_2O$        | in example 22                                      |
| $Na_2PO_4 \cdot ay \cdot 10H_2O$ | in examples 17, 21, 24, 27,<br>28, 31 to 33 and 35 |
| $K_3PO_4$                        | in examples 15 and 29                              |

10 Neutralizing agent (termed "acid" in the table)

|    |                                                                  |     |                              |
|----|------------------------------------------------------------------|-----|------------------------------|
| 10 | HCOOH                                                            | 85% | in examples 12 and 14        |
|    | CH <sub>3</sub> COOH                                             | 60% | in examples 11, 15 to 19, 21 |
|    | C <sub>2</sub> H <sub>5</sub> COOH                               | 60% | to 23, 25, 26, 30 and 35     |
|    | H <sub>2</sub> SO <sub>4</sub>                                   | 10% | in example 20                |
| 15 | H <sub>3</sub> PO <sub>4</sub> ,<br>NaHSO <sub>4</sub>           | 20% | in example 27                |
|    | KHSO <sub>4</sub>                                                |     | in example 24                |
|    | HCl                                                              |     | in example 28                |
|    | NaH <sub>2</sub> PO <sub>4</sub> ·2H <sub>2</sub> O              | 10% | in example 29                |
|    | KH <sub>2</sub> PO <sub>4</sub>                                  |     | in example 33                |
|    | (NH <sub>4</sub> ) <sub>2</sub> HPO <sub>4</sub>                 |     | in examples 13, 36 and 37    |
| 20 | (CH <sub>3</sub> NH <sub>2</sub> ) <sub>2</sub> HPO <sub>4</sub> |     | in example 34                |
|    |                                                                  |     | in example 31                |
|    |                                                                  |     | in example 32                |

Some of the dyebaths contained additionally sodium 3-nitrobenzene-1-sulfonate as a mild oxidizing agent, i.e.

2 parts in examples 13, 28, 26, 33 and 37

3 parts in examples 14, 15, 22, 23, 24, 31, 34, 35, 36

4 parts in examples 11, 12, 27 and 32

### 5 parts in example

Further, a carrier was used for the disperse dyes in the following instances:

30 12 parts of a dichlorobenzene } in Examples 11

|    |                                                                                                                                                                                                                       |                                                                             |
|----|-----------------------------------------------------------------------------------------------------------------------------------------------------------------------------------------------------------------------|-----------------------------------------------------------------------------|
| 35 | 1.2 parts of a highly sulphonated castor oil<br>10 parts of methyl salicylate<br>1 part of a highly sulphonated castor oil<br>10 parts of a mixture of equal parts of dimethyl terephthalate and benzoic acid anilide | in Examples 11, 12, 16, 29 and 32<br>in Examples 14 and 15<br>in Example 36 |
| 40 | 4 parts of para-chlorophenoxy-ethyl acetate<br>1 part of the compound $(C_6H_{10})_2=C_6H_3-(OC_2H_4)_{30}-O-CH_2-COO Na$                                                                                             | in Examples 27, 30, 31 and 33                                               |

The disperse dyes were applied in the form of dye preparations of the following composition:

### 35 percent Dye

### 35 percent Sodium dinaphthylmethane

15 percent Sodium cetyl su

15 percent Sodium sulfate  
The dyeing process was phased as follows: 30 minutes for  
50 heating up to the dyeing temperature for the cellulosic component of the blend; 60 minutes at the dyeing temperature for the cellulosic component; cooling and addition of the acid and the disperse dye; 30 minutes for heating up to the dyeing temperature for the polyester component; 1 hour at the dyeing temperature for the polyester component of the blend.

TABLE

| No. of Example | Water (parts) | Reactive dye (parts) | Alkali (parts) | Salt (parts) | Dyed at (deg.) | Acid (parts) | Disperse dye | Preparation (parts) | Dyed at (deg.) | Shade            |
|----------------|---------------|----------------------|----------------|--------------|----------------|--------------|--------------|---------------------|----------------|------------------|
| 11.....        | 2,000         | 1.5 ①                | 0.55           | 80           | 85             | 2.3          | ②            | 3                   | 95-100         | Orange yellow.   |
| 12.....        | 2,000         | 1.5 ①                | 7              | 80           | 85             | 10.2         | ②            | 3                   | 95-100         | Do.              |
| 13.....        | 1,000         | 1 ②                  | 0.6            | 40           | 85-90          | 4.7          | ②            | 2                   | 130            | Red.             |
| 14.....        | 1,500         | 1 ②                  | 7              | 60           | 60-65          | 5.5          | ⑦            | 1.8                 | 95-100         | Yellow.          |
| 15.....        | 1,500         | 1 ②                  | 8.4            | 60           | 60-65          | 7.5          | ②            | 1.5                 | 95-100         | Violet.          |
| 16.....        | 1,500         | 8 ②                  | 9              | 60           | 65             | 13.0         | ②            | 9                   | 95-100         | Black.           |
| 17.....        | 1,500         | 1 ②                  | 15             | 60           | 70             | 7.5          | ②            | 2                   | 125-130        | Grey.            |
| 18.....        | 1,500         | 1.5 ③                | 9.5            | 60           | 50             | 11.3         | ②            | 1.5                 | 125-130        | Greenish yellow. |
| 19.....        | 1,200         | 1 ②                  | 11.3           | 50           | 50             | 11.3         | ②            | 1.5                 | 125-130        | Yellow.          |
| 20.....        | 1,500         | 1.5 ③                | 9.5            | 70           | 50             | 14.0         | ②            | 1.5                 | 125-130        | Orange.          |
| 21.....        | 2,000         | 1.5 ④                | 18             | 80           | 40-45          | 9.0          | ③            | 1.5                 | 125-130        | Yellow.          |
| 22.....        | 1,500         | 1 ④                  | 19             | 60           | 45-50          | 10           | ⑥            | 1.5                 | 125-130        | Blue.            |
| 23.....        | 1,500         | 1 ⑤                  | 14             | 60           | 85-90          | 9.8          | ③            | 1.5                 | 125-130        | Do.              |
| 24.....        | 1,500         | 1 ⑤                  | 15             | 60           | 40             | 28.5         | ②            | 1.5                 | 125-130        | Do.              |
| 25.....        | 1,500         | 1.5 ④                | 7              | 70           | 85             | 13.2         | ②            | 2                   | 125-130        | Turquoise blue.  |
| 26.....        | 1,500         | 1.5 ⑤                | 7.0            | 60           | 85-90          | 9.1          | ②            | 1.5                 | 125-130        | Do.              |
| 27.....        | 2,000         | 1 ⑤                  | 16.0           | 80           | 85-90          | 38.0         | ⑦            | 2                   | 95-100         | Yellow.          |
| 28.....        | 1,000         | 1 ①                  | 10.0           | 40           | 85-90          | 4.8          | ②            | 2                   | 125-130        | Orange-yellow.   |
| 29.....        | 2,500         | 1 ⑥                  | 11.0           | 100          | 85-90          | 12.5         | ⑥            | 1.8                 | 95-100         | Blue/yellow.     |
| 30.....        | 1,500         | 1.5 ②                | 8.0            | 60           | 60             | 17.5         | ④            | 3                   | 95-100         | Yellow.          |
| 31.....        | 1,500         | 2 ④                  | 15.0           | 60           | 85-90          | 13.6         | ③            | 2                   | 95-100         | Blue.            |
| 32.....        | 2,000         | 1 ①                  | 15.0           | 80           | 85-90          | 51.3         | ⑦            | 2                   | 95-100         | Orange-yellow.   |
| 33.....        | 1,000         | 1 ②                  | 15.0           | 40           | 85-90          | 27.5         | ④            | 2                   | 95-100         | Red.             |
| 34.....        | 1,500         | 1 ②                  | 1.2            | 60           | 85-90          | 5.9          | ④            | 2                   | 125-130        | Orange-red.      |
| 35.....        | 1,500         | 1 ②                  | 15             | 70           | 85-90          | 7.5          | ⑧            | 2                   | 125-130        | Red.             |
| 36.....        | 1,500         | 1 ⑦                  | 0.9            | 70           | 85-90          | 7.0          | ②            | 2                   | 95-100         | Green/red.       |
| 37.....        | 1,000         | 4 ⑦                  | 5.0            | 40           | 85-90          | 29.5         | ⑦+⑧          | 4                   | 125-130        | Green.           |

## 11

The reactive or disperse dyes employed in the foregoing examples have the following constitution.

## 21. 1-(4'-Hydroxyphenylazo)-4-phenylazobenzene

22.



## 23. Potassium 1-(2' chloro-6'-methylphenyl)3-methyl-4-(2'-methoxy-5'-sulfato-ethylsulfonyl-phenylazo)-5-pyrazolone-4'-sulfonate

## 24. The copper complex compound of potassium 1-hydroxy-2-(2'-hydroxy-4'-vinylsulfonylphenylazo)-8-acetylaminoanthracene-3,6-disulphonate

## 25. 1-Hydroxy-4-(2'ethoxycarbonyl-ethylamino)-anthraquinone

## 26. Potassium 1-hydroxy-8-amino-2,7-bis(sulphato-ethylsulfonylphenylazo)-naphthalene-3,6-disulphonate

## 27. Mixture of 45 percent of 2,4-dinitro-6-bromo-2'-acetylamino-5'-ethoxy-4'-N,N'-bis-(acetoxymethyl)-amino-1,1'-azobenzene, 20 percent of 2,4-dinitro-6-chloro-2'-acetylamino-5'-methoxy-4'-N,N'-bis-(acetoxymethyl)-amino-1,1'-azobenzene, 25 percent of 4-nitro-2-bromo-4'-N-acetoxymethyl-n-cyanethylamino-1,1'-azobenzene and 10 percent of 4-nitro-2,6-dibromo-4'-N-methyl-N-cyanethylamino-1,1'-azobenzene

## 28. The 2:1 mixed chromium-cobalt complex of sodium-1-hydroxy-2-(2'-hydroxy-6'-nitronaphthyl-1'-azo)-6-(4'-chloro-6'-amino-1', 3'', 5''-triazinyl-2''-amino)-naphthalene-3,4'-disulphonate.

## 29. Mixture of 41 percent of 2,6-dichloro-4-nitro-4'-N-cyanethyl-N-acetoxymethylamino-1,1'-azobenzene, 49 percent of 1,5-diamino-2-bromo-4,8-dihydroxyanthraquinone and 10 \*\*percent of 2-cyano-4-nitro-4'-N-ethyl-N-cyanethylamino-1,1'-azobenzene.

## 30. Sodium 1-(2', 5'-dichlorophenyl)-3-methyl-4-[3''-(4'', 6''-dichloro-1'', 3'', 5''-triazinyl-2''-amino)-phenylazo]-5-pyrazolone-4', 6''-disulphonate

## 31. 5-Benzoylamino-1,9-thiazolanthrone

## 32. 4-Nitro-9-acridone

## 33. Sodium 1-hydroxy-2-phenylazo-6-(4'', 6''-dichloro-1'', 3'', 5''-triazinyl-2''-amino)-naphthalene-3,2'-disulphonate

## 34. Sodium 2-[4-(2'', 3''-dichloroquinoxaly-6''-carbonyl-amino)-2'-methyl-phenylazo]-naphthalene-4,8-disulphonate



## 36. Sodium 1-amino-4-[3'-(4'', 6''-dichloro-1'', 3'', 5''-triazinyl-2''-amino)-phenylamino]-anthraquinone-2,4'-disulphonate.

## 37. Sodium 1-amino-4-(3'-trichloropyrimidylamino-phenylamino)-anthraquinone-2,4'-disulphonate.

## 38. 1:1 Mixture of 1,5-diamino-4,8-dihydroxy-2-(4'-hydroxyphenyl)-anthraquinone and 1,5-diamino-4,8-dihydroxy-2-(4'-methoxyphenyl)-anthraquinone

## 39. Sodium 1-amino-4-4'[-N(2'', 3''-dichloroquinoxaly-6''-carbonyl)-N-methyl-amino-methyl]-phenylamino-} anthraquinone 2,3'-disulphonate

## 40. Disodium salt of copperphthalocyanine-(3)-disulfonic acid-sulfonic acid/amide-sulfonic acid-[3'-(4''-amino-6''-chloro-1'', 3'', 5''-triazinyl-2''-amino)-6''-sulphophenylamide]

## 41. 1,4-Diamino-anthraquinone-2,3-dicarboxylic acid -(3'-methoxypropylimide.)

## 42. Disodium salt of copperphthalocyanine-(3)-disulfonic acid-sulfonic acid/amide-sulfonic acid -(3'-trichloropyrimidylaminophenylamide)

## 12

## 43. Sodium 4-trichloropyrimidylamino-4'-(3''-methyl-4''-(2''-methylphenylazo)-5''-pyrazolonyl-1')-stilbene-2,2', 5''-trisulphonate



## 45. Bis-copper complex compound of sodium 1,6-dihydroxy-2-(2'-hydroxy-5'-trichloropyrimidylaminophenylazo)-5-(1''-hydroxynaphthyl-2''-azo)-naphthalene-3, 3', 4'', 6''-tetrasulphonate

## 46. 2-Cyano-4-nitro-4'-N-β-cyanethyl-N-β-acetoxymethyl-amino-1,1'-azobenzene

15



20

47.

Nickel-phthalocyanine

(SO3Na)3

SO3-NH-C6H4-N=N-C6H2(O)-C6H2(CH3)-N

25

-C6H4-NH-trichloropyrimidyl

42

We claim:

1. A process for dyeing a blend of natural or regenerated cellulosic fiber component and linear polyester fiber component with reactive dye and disperse dye comprising exhaustion dyeing the cellulosic component first with the reactive dye in a dyebath in the presence of at least one neutral salt and of not more than 20 grams of basic fixing agent per liter of dyeliqour at a temperature in the range of 40° to 100° C. and at a pH in the range of 8.5 to 13, then adjusting the pH to from 4 to 7, adding the disperse dye to the dyeliqour and dyeing the polyester component of the blend.

2. A process according to claim 1 wherein the basic fixing agent is from 0.2 to 1.2 grams of sodium or potassium hydroxide per liter of dyeliqour.

3. A process according to claim 1 wherein the basic fixing agent is from 2 to 20 grams of sodium or potassium carbonate or trisodium phosphate per liter of dyeliqour.

4. A process according to claim 1 wherein dyeing is carried out at a goods-to-liquor ratio of 1:4 to 1:30.

45 5. A process according to claim 1 wherein the temperature for dyeing the cellulosic component is from 80° to 95° C.

6. A process according to claim 1 wherein the reactive dye bears a dihalogenopyrimidyl or trihalogenopyrimidyl group.

7. A process according to claim 1 wherein the reactive dye bears a monohalogenotriazinyl or a dihalogenotriazinyl group.

8. A process according to claim 1 wherein the reactive dye bears a 2,3-dihaloquinoxaly-6-carbonyl, -6-sulphonyl- or -6-aminocarbonyl group.

9. A process according to claim 1 wherein the reactive dye bears a sulphatoethylsulphonyl or a vinylsulphonyl group.

10. A process according to claim 1 wherein the pH value is reduced to from 4 to 7 by adding an organic lower aliphatic acid to the dyebath.

60 11. A process according to claim 1 wherein the pH value is reduced to from 4 to 7 by adding to the dyebath a phosphate of the formula MeH2PO4, wherein Me is an alkali metal, ammonium or a low-molecular alkylammonium radical.

12. A process according to claim 1 wherein the dyebath is adjusted to a pH of from 5 to 6.5 before adding the disperse dye thereto.

65 13. A process according to claim 1 wherein the polyester component of the blend is dyed at from 95° to 100° C. or at the boil in the presence of a carrier for dyeing linear polyester fiber.

70 14. A process according to claim 1 wherein the polyester component is dyed in the temperature range of from 110° to 140° C. under pressure in the absence of carrier for dyeing linear polyester fiber.

\* \* \* \* \*

UNITED STATES PATENT OFFICE  
CERTIFICATE OF CORRECTIONPatent No. 3,617,168Dated November 2, 1971Inventor(s) ROLF MACK

It is certified that error appears in the above-identified patent and that said Letters Patent are hereby corrected as shown below:

Column 1, line 7, "timesaving" should read --time-saving--; line 27, "ph" should read --pH--; line 57, "phrimidyl" should read --pyrimidyl--; line 64, in the formula, "G-X-Z" should read --C-X-Z--. Column 2, line 4, "or -SO<sub>2</sub>-CH" should read --or -SO<sub>2</sub>-CH=--; line 6, "-CH<sub>2</sub>-O-SO<sub>3</sub>H" should read -- -CH<sub>2</sub>-O-SO<sub>3</sub>H;--; line 7, "dichloroquinoxalyl16-" should read --dichloroquinoxalyl-6--; line 27, "-CH<sub>2</sub>O-SO<sub>3</sub>H-" should read -- -CH<sub>2</sub>-O-SO<sub>3</sub>H- --; line 28, "-SO<sub>2</sub>-CH CH<sub>2</sub>" should read -- -SO<sub>2</sub>-CH=CH<sub>2</sub>--; line 49, "for" should read --from--; line 60, "The disperse" should start a new paragraph. Column 3, line 66, "(CH<sub>3</sub>)<sub>2</sub>NHB?<sub>2</sub>," should read --(CH<sub>3</sub>)<sub>2</sub>NH<sup>+</sup><sub>2</sub>,--; "neutralized an" should read --neutralized and--. Column 4, line 68, "NaH<sub>2</sub>PO<sub>4</sub>·2H<sub>2</sub>O" should read --NaH<sub>2</sub>PO<sub>4</sub>·2H<sub>2</sub>O--. Column 5, line 12, "Na<sub>3</sub>PO<sub>4</sub>·1OH<sub>2</sub>O" should read --Na<sub>3</sub>PO<sub>4</sub>·1OH<sub>2</sub>O--; line 25, in the formula, "<sub>NH-C</sub><sup>//</sup>" should read --<sub>NH-C</sub><sup>//</sup>--; "SO<sub>3</sub>NA" should read --SO<sub>3</sub>Na--; line 37, "suphate" should read --sulphate--; line 49, "suphate" should read --sulphate--; line 69, delete "methanedisulphonate". Column 6, line 3, "7" should read --⑦--; line 8, after the formula insert --⑧--; line 11, "5" should read --⑤--; "1" should read --①--; line 25, in the formula, "SO<sub>3</sub>Na" should read -- SO<sub>3</sub>Na--; line 42, "10" should



read --⑩--; line 54, "3nitrobenzenesulphonate" should read --3-nitrobenzenesulphonate--; line 72, "12" should read --⑫--.

PO-1050  
(5/69)

UNITED STATES PATENT OFFICE  
CERTIFICATE OF CORRECTION

Patent No. 3,617,168

Dated November 2, 1971

Inventor(s) ROLF MACK

It is certified that error appears in the above-identified patent and that said Letters Patent are hereby corrected as shown below:

Column 7, line 16, in the formula, "N--NH-" should read -- -N--NH- --; line 20, "and entered" should read --are entered--; line 29, "4" should read -- ④ --; line 54, in the formula, "NH-trichloropyrimidyl" should read -- -NH-trichloropyrimidyl--; line 55, "1" should read -- ① --; line 67, "4"

should read -- ④ --; line 70, in the formula, "  " should read --H<sub>2</sub>--; line 77, in the formula "  " should read --  --


 NH - C 
 --. Column 8, line 21, in the formula,  
 " 
 SO2-C2H4-O-SO3K" should read -- 
 SO2-C2H4-O-SO3K --;  
 line 33, "6" should read -- ⑥ --; line 50, in the formula,  
 " 
 Cl" should read -- 
 Cl --; line 63, "18"

should read -- 18 --. Column 9, line 17, "ethoxyanthraquinone" should read --ethoxyanthraquinone--; line 19, "20" should read -- 20 --; line 25, "The following" should start a new paragraph. Column 10, line 7, " $\text{Na}_3\text{PO}_4 \cdot 10\text{H}_2\text{O}$ " should read -- $\text{Na}_3\text{PO}_4 \cdot 10\text{H}_2\text{O}$ --; line 33, "nonated" should read .

UNITED STATES PATENT OFFICE  
CERTIFICATE OF CORRECTION

Patent No. 3,617,168

Dated November 2, 1971

Inventor(s) ROLF MACK

It is certified that error appears in the above-identified patent and that said Letters Patent are hereby corrected as shown below:

--nated--; example 32, in the table, under "Acid (parts)", "51.3" should read --15.3--. Column 11, line 13, in the formula, "NH-trichloropyrimidyl" should read -- -NH-trichloropyrimidyl--; line 14, ")3-methyl-4-(2" should read --)-3-methyl-4-(2"--; line 29, "yethyl-n-" should read --yethyl-N- --; line 39, "%%percent" should read --percent--; line 40, "1 1'" should read --1,1'--; line 50, before the formula, insert "35."; line 64, "4- 4'[-N" should read --4-{4'-[N- --; line 66, "2,3'-" should read -- -2,3'--. Column 12, line 19, in the formula, "



should read -- --.

Signed and sealed this 19th day of March 1974.

(SEAL)

Attest:

EDWARD M. FLETCHER, JR.  
Attesting Officer

C. MARSHALL DANN  
Commissioner of Patents